

## UNITED STATES PATENT OFFICE.

JACQUELINE KNOLLEMA, OF SAN FRANCISCO, CALIFORNIA.

## ART OF DECORATING FABRIC.

No Drawing.

Application filed July 20, 1925. Serial No. 44,906.

This invention relates to a certain new and useful improvement in the art of decorating fabric and has particular reference to the application to handkerchiefs and the like, 5 of an ornamental border comprising a gold or silver edging.

The principal object of this invention is to perfect a solution from certain ingredients by which the handkerchiefs and the like, 10 will be ornamented with a border of gold or silver that will produce a permanent flexible ornamentation that will not become hardened or be displaced from the handkerchief or the like when the fabric is washed. 15 The application of the gold border to the handkerchief prevents the edges of the same from ravelling and I thereby eliminate the hemstitching which is usually employed.

In carrying out my process to realize my 20 solution, I take a quantity of gum, which in the trade is termed "varnish gum," of approximately 14% proportion, then mix with the melted varnish gum a 50% proportion of linseed oil and China-wood oil, then 25 add to this mixture 35% of turpentine and 1% of either silver or gold bronzing powder or paint.

The ingredients as described are thoroughly mixed in a suitable receptacle and the 30 preparation can then be readily applied to fabric, such as, handkerchiefs for realizing the desired ornamental and artistic effect of a silver or gold border.

Although an ornamental border has been 35 specified, it is, nevertheless, to be understood that the other parts of the handkerchief or the like can be likewise treated for the pur-

pose of realizing any desired artistic representation.

By experience I have found that the use 40 of linseed oil and China-wood oil accounts for the flexibility of the preparation when it is applied to the fabric for the purpose of ornamentation, and I have further ascertained that the varnish gum serves the 45 purpose of making the preparation adhere to the fabric. Furthermore, the danger of displacement of the silver or gold preparation from the handkerchief or the like is eliminated when the same is washed. 50

While I have specified the ingredients that are preferably employed, it is to be understood that any other desired ingredients having the same properties as the elements specified can be utilized without departing from the spirit of the invention or the scope of the claim. 55

Obviously, changes relative to the proportions of the ingredients used may likewise be made without departing from the principle of the invention or the scope of the subjoined claim. 60

Having thus described my invention, I claim:—

A composition for preventing an unravelling the edges of handkerchiefs and like fabrics and serving to ornament the same comprising 14% varnish gum, 25% linseed oil, 25% China-wood oil, 35% turpentine, and 1% of a bronzing powder. 65 70

In testimony whereof I affix my signature.

JACQUELINE KNOLLEMA.